

## UNITED STATES PATENT OFFICE

1,974,861

## PRODUCTION OF LEATHER

Giorgio Chiera, Torino, Italy, assignor to the firm  
J. R. Geigy A. G., Basel, Switzerland

No Drawing. Application April 27, 1934, Serial  
No. 722,815. In Germany May 11, 1933

2 Claims. (Cl. 149—2)

As is well known it is necessary to subject animal skins, before tanning, to a preparatory treatment for separating the epidermis and the under-skin. After liming and after removal of the hair-bearing outer layer the corium is left in a strongly swollen, "plump and full" condition, in which it still encloses residues of the liming agent. If the skin is tanned whilst it is in this swollen condition it yields only a poor leather. By bathing or drenching, for example, with a fermented infusion of bran or dung or even with pure enzymes, the swelling is reduced and the skin becomes flaccid or "fallen"; whilst it is in this condition the residual impurities, even those enclosed within the skin, can be removed easily by mechanical means.

At the same time the surface of the skin requires the favourable condition required for the tanning operation, this being recognized by the slippery feel of the skin. The softness and suppleness of the leather obtained after tanning is dependent not only on the known specific action of the liming agent but also largely on the extent to which the liming agent and the impurities are removed.

This invention is based on the observation that a pre-treatment of the skins, with a washing and emulsifying agent obtainable according to German Specification No. 506,338 from a pyrophosphate and glue, gelatin, proteins, saponin, casein and so on, prior to tanning, is remarkably suitable for the purpose of rendering the leather very soft and supple. If an animal hide which has been prepared for tanning in the usual manner is treated, before or after the bathing or drenching operation, in a bath containing a washing and emulsifying preparation obtainable according to the aforesaid specification, there is obtained after tanning a leather which is much softer and more supple than that which

is obtained with the aid of the hitherto usual bathing processes. Thus a treatment in accordance with the invention may replace the hitherto usual bathing processes. The duration of the treatment will vary according to the effect which is desired and according to the concentration of the bath.

The following example illustrates the invention, the parts by weight:—

Skins which have been prepared in the beamhouse in the usual manner by liming and bathing are placed in water having a temperature of 35–40° C., on the reel or in the drum and moved for 1–1½ hours with the addition of 1–1½ per cent of a mixture of 2 parts of neutralized sodium pyrophosphate and 1 part of casein. The skins are then washed and tanned in the usual manner. The proportion of the mixture of pyrophosphate and casein which is used depends upon the origin of the skins and must be greater the higher the content of the skins in fat.

Instead of casein, it may be possible to use in this example any natural, vegetable or animal albumen such as glue, gelatin, a protein, saponin and so on.

What I claim is:—

1. An improvement in the production of leather, consisting in subjecting the skin, in the course of the treatment preparatory to tanning, to a treatment with a solution of a washing and emulsifying agent obtainable from a pyrophosphate and any natural, vegetable or animal albumen.

2. An improvement in the production of leather, consisting in subjecting the skin, in the course of the treatment preparatory to tanning, to a treatment with a solution of a washing and emulsifying agent obtainable from sodium pyrophosphate and casein.

GIORGIO CHIERA. 95